

## UNITED STATES PATENT OFFICE

2,167,301

## ALLOY CAST IRON

Edwin A. Jones, Jackson, and Arthur H. Dierker,  
Columbus, Ohio, assignors to Globe Iron Company,  
Jackson, Ohio, a corporation

No Drawing. Application March 23, 1938,  
Serial No. 197,726

4 Claims. (Cl. 75—126)

Our present invention relates to an improvement in alloy cast iron, in which silicon and chromium are the principal alloying agents, and in which the silicon, in the various proportions in which it may be used with reference to the chromium, is always in substantial excess of the chromium content.

We have found that alloys prepared in accordance with our invention, have high wear and heat-resisting properties, and exhibit unusual resistance to scaling, warping and growth at elevated temperatures.

We have further found that such alloy cast irons are machinable at Brinell hardness far in excess of that at which cast irons or steels are considered to be unmachinable.

Further, our alloy cast iron can be produced from low cost materials, in furnaces of the cupola type, which are recognized as being the lowest cost type of furnace in common use today, and by labor which does not require to be highly skilled.

Cast iron is generally considered to contain the following materials substantially within the ranges indicated, namely—

|              | Per cent     |
|--------------|--------------|
| Total carbon | 2.50 to 3.70 |
| Silicon      | .80 to 3.00  |
| Manganese    | .40 to 1.20  |
| Sulphur      | Under 0.20   |
| Phosphorus   | Under 1.00   |

Where any of the elements exceed the maximum amounts indicated, the excess of the amount of such element usually required to produce an iron of normal properties, is considered an alloying element.

In the alloy cast iron of our invention, we use silicon in excess of the amount required to produce a good quality of cast iron, as an alloying agent to secure properties not found in unalloyed irons, and we also use chromium as an alloying agent, but in the compositions of our alloy we maintain the silicon content always in excess of the chromium content by a substantial amount.

Despite its hardness, our alloy contains as cast free carbon in the form of graphite flakes or nodules, and is thus definitely not a steel, and should not be confused with steels containing silicon and chromium.

With the foregoing explanation in mind, one of the principal objects of our invention is to provide an alloy cast iron having high wear and heat resisting properties and unusual resistance to scaling, warping and growth at elevated temperatures.

A further object is to provide an alloy cast iron of great hardness, which is machinable at unusually high Brinell hardness, and without the use of lubricants.

A further object is to provide an alloy cast iron comprising silicon and chromium as the principal alloying agents, with the silicon in excess of the chromium, and having free graphite, the alloy being characterized by high resistance to wear, and to scaling, warping and growth at elevated temperatures, and being machinable at hardnesses far beyond those of cast irons.

Still another object of our invention is to provide an alloy cast iron of the characteristics set forth above, and having a relatively low melting point and low shrinkage characteristics, such that good castings of intricate and thin sections can be produced with ordinary foundry facilities.

A further object is to provide an alloy cast iron having the various qualities and characteristics referred to, which is capable of production in cupola furnaces at relatively low cost, and without requiring labor of anything more than ordinary skill.

In producing our alloy cast iron, we prefer that it contain constituents within the following table, namely—

|            | Per cent   |
|------------|------------|
| Silicon    | 3.05-10.00 |
| Chromium   | 0.60- 8.00 |
| Manganese  | 0.20- 3.00 |
| Phosphorus | Under 0.30 |
| Sulphur    | Under 0.20 |
| Carbon     | 1.80- 3.20 |

While the percentages of the various materials within the ranges indicated may vary, in all cases we keep the silicon content in excess of the chromium by a substantial amount. The presence of the relatively high silicon content with regard to the chromium in our alloy, we believe, lowers the solubility of the carbon in the iron at room temperatures, and hence, as the iron cools from

the molten condition, carbon is precipitated from solution in the form of graphite, which is distributed substantially uniformly throughout the body of the metal in the form of small flakes or nodules.

The alloy can be produced from relatively low cost raw materials and in simple and economical types of melting units, by workmen of no more than ordinary skill. As illustrative, alloy steels require for their production, the use of the electric furnace, the open hearth furnace, or the crucible furnace. All of these types of furnaces are expensive to build, maintain and operate. Our alloy, on the other hand, can be produced in the cupola type furnace which, as recognized in the industry, is the type of furnace which is the cheapest per unit of capacity, in common use. It is not only less expensive in initial cost, than the other types of furnaces referred to, but is also cheaper to maintain and operate.

Examples of a number of compositions of our alloy are given in the tables which follow, in which tables various specimens have been tested against other cast irons.

We give below some results of wear tests, as well as tests of other physical properties, and a few compositions of the alloy of our invention. The wear tests were made by holding the specimen under a weight of 1380 grams on the table of a Dorry machine, a constant stream of washed silica sand being fed to the table during the test. At the end of 6000 revolutions, the specimen was moved and weighed, and the weight loss due to wear was noted. The physical properties were determined by standard A. F. A. methods.

| Specimen No.                      | 70     | 71     | 2352   | 2395   | 2423   | 2423         |
|-----------------------------------|--------|--------|--------|--------|--------|--------------|
| 40 Analysis:                      |        |        |        |        |        |              |
| T. C.                             | 3.30   | 3.10   | 2.52   | 3.17   | 2.21   | Heat treated |
| Si.                               | 2.40   | 1.73   | 4.23   | 3.05   | 5.30   |              |
| Mn.                               | .65    | .94    | .60    | .50    | .63    |              |
| P.                                | .18    | .16    | .11    | .056   | .084   |              |
| S.                                | .11    | .13    | .065   | .065   | .052   |              |
| Cr.                               |        |        | 2.20   | .96    | 2.98   |              |
| 45 Brinell hardness No.           | 170    | 217    | 255    | 255    | 341    | 388          |
| Transverse strength pounds        | 2,560  | 3,230  | 2,950  | 3,290  | 2,120  |              |
| Deflection inches                 | .292   | .270   | .190   | .282   | .137   |              |
| Tensile strength lbs. per sq. in. | 29,200 | 43,000 | 34,700 | 42,800 | 32,000 | 43,000       |
| Wear loss grams                   | 5.19   | 3.85   | 1.931  | -----  | 2.07   | 1.67         |

50 In the foregoing table of tests, specimen No. 70 is a typical medium strength cast iron, while No. 71 is a high strength cast iron. Both were made in regular production in a commercial foundry. The other specimens are alloys of our invention. The heat treated specimen No. 2423, is of the same composition as the specimen of that same number in the table, but not designated as heat-treated. The heat treatment consisted of normalizing at 1800 deg. F. and drawing at 1300 deg. F.

The above data shows that the alloy iron, despite its high hardness, has strength and toughness comparable to a good grade of high test iron.

65 A remarkable feature of our alloy is that it can be machined at unusually high Brinell hardness. Cast iron is ordinarily considered unmachinable when it has a Brinell hardness of more than 280. All of the given examples of our alloy, however, even though they tested up to 388 Brinell, were readily machinable, and indeed, we have machined specimens of our alloy having a Brinell hardness of 415.

The superior resistance of our alloy to growth

and scaling at elevated temperatures, is indicated in the following table.

The specimens used were heated under identical conditions, in a gas fired furnace for six cycles. Each cycle consisted of bringing the furnace to 1650 deg. F., holding it for five hours, and then allowing to cool over night. The results of the test are given below.

| Specimen No.        | 134-3 | 219-6 | 116-1 | 10 |
|---------------------|-------|-------|-------|----|
| Analysis:           |       |       |       |    |
| T. C.               | 2.13  | 2.80  | 3.44  |    |
| Si.                 | 5.73  | 2.30  | 2.25  |    |
| Mn.                 | .37   | .53   | .56   |    |
| P.                  | .05   | .27   | .43   |    |
| S.                  | .02   | .08   | .06   | 15 |
| Cr.                 | 4.16  |       |       |    |
| Scale loss, percent | 2.00  | 8.87  | 10.70 |    |
| Growth, percent     | .07   | 1.74  | 5.82  |    |

In this table, specimen 134-3 is an alloy of our invention, while specimen 219-6 is a high strength cast iron, and specimen 116-1 is a soft cast iron. The scale loss and the growth of our alloy are both remarkably low, as indicated in the table.

25 In addition to the qualities of unusual high hardness, and high wear and heat-resistance, our alloy exhibits the further quality of relatively small shrinkage during solidification of the metal from the molten state, and in addition, has a melting point very much lower than alloy steels. Hence the alloy possesses excellent casting properties, such indeed, that with ordinary foundry facilities, sound castings of intricate and thin sections can be made.

30 We are aware that steels containing silicon and chromium are known in the art, but our alloy possesses characteristics which distinctly differentiate it from such steels, such for instance, as its low production cost; its machinability; its silicon content in excess of the chromium; and its brittleness as compared to workability of steel; also ease of casting to shape as compared to steel.

On the other hand, the ability of our alloy to be machined at Brinell hardness far greater than that of cast irons, and its unusually high heat resistance and wear resistance, give it qualities unpossessed by cast irons heretofore known in the art with which we are acquainted.

It will be understood that our alloy may be heat-treated subsequent to casting by one of the accepted methods for ferrous alloys; i. e., annealing, either at a temperature above or below the critical; normalizing from a temperature above or below the critical; quenching from a temperature above the critical and drawing at some suitable temperature below the critical.

While the foregoing description sets out a number of specific embodiments of our invention, it will be understood that various changes in proportions of the elements constituting our alloy may be made within the scope of the appended claims. It will further be understood that the foregoing description has been given for purposes of illustration of our invention, and that no undue limitations should be deduced therefrom, but that the claims should be broadly construed within the limitations of the prior art.

Having thus described our invention what we claim as new and desire to secure by United States Letters Patent is:

1. An alloy cast iron, having silicon in proportions greater than chromium, and in which a substantial part of the carbon is in the form

of free graphite, said alloy containing silicon 4.23% to 10.00%; chromium 0.6% to 8.00%; manganese 0.20% to 3.00%; phosphorus under 0.30%; sulphur under 0.20%; carbon 1.80% to 3.20%, and the balance iron.

2. An alloy cast iron containing silicon about 4.23%; manganese about .60%; phosphorus about .11%; sulphur about .065%; chromium about 2.20%, total carbon about 2.50%, and the balance iron, said alloy being characterized by high wear and heat resistance.

3. An alloy cast iron containing silicon about 5.30%; manganese about .63%; phosphorus

about .084%; sulphur about .052%; chromium about 2.98%, total carbon about 2.20%, and the balance iron, said alloy being characterized by high wear and heat resistance.

4. An alloy cast iron containing silicon about 5.73%; manganese about .37%; phosphorus about 0.05%; sulphur about .02%; chromium about 4.16%, total carbon about 2.13%, and the balance iron, said alloy being characterized by high wear and heat resistance.

10

EDWIN A. JONES.  
A. H. DIERKER.